

# UNITED STATES PATENT OFFICE.

GUSTAV JACOB LESSER, OF FRANKFORT-ON-THE-MAIN, GERMANY,  
ASSIGNOR TO ROBERT E. LESTER, OF NEW YORK, N. Y.

## PROCESS OF COLORING GLUE.

SPECIFICATION forming part of Letters Patent No. 276,609, dated May 1, 1883.

Application filed March 29, 1883. (No specimens.)

*To all whom it may concern:*

Be it known that I, GUSTAV JACOB LESSER, of Frankfort-on-the-Main, Germany, have invented an Improved Process of Coloring Glue, of which the following is a specification.

Common black or dark glue, while possessing all the adhesive and other essential qualities of fine colored glue, has heretofore, owing to its color, been confined in its use to such purposes in the arts as where color was not essential.

The object of this invention is to color such glue so that it is both refined and tinted, and may be used for various purposes in the arts. It will be especially applicable in the manufacture of sizing and finishing compounds for paper-hangings, compounds for the manufacture of elastic rolls, for glue and size compounds for finishing yarns, textile fabrics of silk, cotton, &c., for the manufacture of calcimines and wall-coverings, for glue to be used with colored woods, and for all other purposes where a fine strong colored glue is required.

For coloring common black or dark glue I take a pound and a half of liquid extract of lead and mix it into the water in which the glue has been soaked, as follows: thirteen pounds of glue, sixty-three and a quarter pounds of water. I allow the glue to soak for about twenty-four hours, when I dilute it by a slow fire, and when heated I gradually pour in one and a half pound of the extract of lead and mix it well together.

The extract of lead is a well-known commercial article, and I find it well suited for my purpose; but I do not limit myself to this particular preparation, as there are a large number of neutral and basic compounds of lead that may be so modified as to produce results similar if not identical with the results obtained by the formula above given. Gelatine may be treated instead of glue.

I do not limit myself to the exact proportions or method of mixing herein given, as the same may be varied to some extent without departing from my invention.

Having thus described my invention, what I claim is—

1. The improved colored glue herein described, composed of common glue and a lead compound, substantially as described.
2. The combination of a solution of glue with liquid extract of lead, substantially as described.
3. The process of coloring glue and gelatine herein described by treating a solution of glue or gelatine with a lead solution, as described.

In witness whereof I have hereunto set my hand.

GUSTAV JACOB LESSER.

Witnesses:

F. VOGELER,  
J. GRUND.